

July 29, 1930.

J. A. M. VAN LIEMPT

1,771,974

PROCESS OF COATING BODIES WITH TUNGSTEN

Filed Dec. 2, 1924



Inventor

Johannes Antonius Marie Van Liempt  
By G. T. & J. F. Braudekina  
attorneys

## UNITED STATES PATENT OFFICE

JOHANNES ANTONIUS MARIA VAN LIEMPT, OF EINDHOVEN, NETHERLANDS, ASSIGNOR  
TO N. V. PHILIPS' GLOEILAMPENFABRIEKEN, OF EINDHOVEN, NETHERLANDS

## PROCESS OF COATING BODIES WITH TUNGSTEN

Application filed December 2, 1924, Serial No. 753,452, and in the Netherlands June 28, 1924.

The invention comprises a process of coating bodies with tungsten.

According to the invention the process of coating with tungsten a body consisting of electrically conducting material consists in that a fused tungstate or a mixture of fused tungstates is electrolyzed at such a current density that tungsten is isolated as a coherent layer on the body which is connected as a cathode. Tungstates are compounds of the composition  $nX_2OmWO_3$  if  $n$  and  $m$  are whole numbers and  $X$  is a metal. It has been found that the electrolysis according to the invention can be carried out with very favourable results, if the current density is lower than 100 milliamp. per  $cm^2$  of the surface of the cathode. As a rule it is advisable to start from a tungstate or a mixture of tungstates having a low melting point. According to the invention, preferably a fused alkali tungstate or a mixture of fused alkali tungstates is electrolyzed. Particularly favourable results are obtained in the electrolysis of lithium tungstate ( $Li_2WO_4$ ), but also with other alkali tungstates the electrolysis can be carried out with favourable results.

According to the invention the temperature at which the electrolysis is carried out is preferably over  $900^\circ$  centigrade, as it may occur that below  $900^\circ$  centigrade tungsten nebulae are produced, which do not separate on the cathodes as a solid but remain colloidally dissolved in fusion. It is generally preferable that the temperature at which the electrolysis is carried out should not be too close to the melting point of the tungstate or the mixture of tungstates, because if this temperature difference is too small this would involve a high degree of viscosity of the molten mass, which is injurious to the electrolytic process. The condition herein set up is satisfied, for example, by lithium tungstate ( $Li_2WO_4$ ) which melts at about  $750^\circ$  centigrade but also an eutectic mixture of lithium tungstate ( $Li_2WO_4$ ) and potassium tungstate ( $K_2WO_4$ ) having a melting point of say  $500^\circ$  centigrade or a given mixture of sodium ( $Na_2WO_4$ ) and potassium tungstate ( $K_2WO_4$ ) that melts at about  $650^\circ$  centigrade may be used with advantage but also with other tungstates of the

composition  $nX_2OmWO_3$  favourable results have been obtained.

In the electrolysis care should generally be taken that the fusion is not going to contain too great an excess of  $WO_3$  since it has been found that such an excess of  $WO_3$  may cause an isolation of tungsten bronzes which contain less oxygen than tungstates and correspond to the general formula



These tungsten bronzes are sometimes produced even if the excess of  $WO_3$  is but 5%.

According to the invention the body on which tungsten is precipitated may consist of a single tungsten crystal. The body has been found to increase in this case whilst keeping its one-crystal structure so that an one-crystal body can thus be produced which is larger than the original one. For this purpose one-crystal wires, rods or the like of tungsten are, during the electrolytic treatment preferably connected as a cathode in front of an anode which surrounds the cathode substantially. Such an anode, may, for example, be cylindrical or it may consist of little rods that are arranged parallel to each other in the shape of a many sided prism.

The invention will be more clearly understood by reference to the accompanying drawing. In a porcelain crucible 1 containing lithium tungstate ( $Li_2WO_4$ ) are arranged two electrodes 2 and 3, one of which, the anode, consists of tungsten whereas the other one, the cathode may be, for example, a body made of copper. The said electrodes are connected with the interposition of a potentiometer whilst 4 is a source of continuous current and 5 a regulating resistance. It is found that a regular isolation of tungsten occurs at the cathode and that the said tungsten rigidly adheres as a coherent layer to the cathode, if between the electrodes a tension of 0.08 volt is supplied and the current density is 75 milliamp. per  $cm^2$ .

If the body that is wished to be sheathed with tungsten consisting of material to which tungsten adheres less readily it is preferable that the body should be first coated with a layer to which tungsten adheres readily.

Thus, for example, it is advisable that a body of iron which is desired to be tungstenized is first coppered and not until then tungstenized. According to the invention bodies consisting of non conducting material may be tungstenized by first coating them with one or more layers of electricity conducting material before the coating with tungsten has been effected. Thus, for example, bodies of non-conducting material may first be coated with graphite, then coppered and finally tungstenized.

When using a cylindrical anode a tungsten one-crystal wire connected as a cathode, having a diameter of 300 microns and being plunged for three centimetres into fused lithium tungstate will within two hours increase in size to the extent of a tungsten one-crystal rod having a diameter of 2 millimetres, if the tension at the electrodes is 0.08 volt and the current density is 100 milliamperes per square centimeter.

What I claim is:

1. A process of coating a body with tungsten which comprises electrolyzing a fused alkaline tungstate at a current density which is lower than 100 milliamperes per square centimeter of the surface of the cathode, the body to be coated being connected as cathode.
2. A process of coating a body with tungsten which comprises electrolyzing a fused alkaline tungstate at a current density which is lower than 100 milliamperes per square centimeter of the surface of the cathode, the body to be coated being connected as cathode and the temperature at which the electrolysis is carried out being over 900° centigrade.

In testimony whereof I affix my signature, at the city of Eindhoven, this 25th day of October, 1924.

JOHANNES ANTONIUS MARIA VAN LIEMPT.

45

50

55

60